

W. H. HOWARD,  
PROCESS OFrecovering SULFUR DIOXID,  
APPLICATION FILED MAY 10, 1918.

1,377,012.

Patented May 3, 1921.



INVENTOR  
*William H. Howard*  
BY  
*Messimer and Austin*  
ATTORNEYS

# UNITED STATES PATENT OFFICE.

WILLIAM H. HOWARD, OF SALT LAKE CITY, UTAH, ASSIGNOR TO AMERICAN SMELTING AND REFINING COMPANY, OF NEW YORK, N. Y., A CORPORATION OF NEW JERSEY.

## PROCESS OF RECOVERING SULFUR DIOXID.

1,377,012.

Specification of Letters Patent.

Patented May 3, 1921.

Application filed May 10, 1918. Serial No. 233,640.

To all whom it may concern:

Be it known that I, WILLIAM H. HOWARD, a citizen of the United States, and resident of Salt Lake City, in the county of Salt Lake 5 and State of Utah, have invented certain new and useful Improvements in Processes of Recovering Sulfur Dioxid, of which the following is a specification.

My invention relates to a process for the 10 recovery of sulfur dioxid as a by-product from the waste gases incident to blowing copper matte in a converter.

Sulfur dioxid has heretofore been recovered as a by-product incident to other metallurgical operations and processes, but in attempting to apply the same processes to waste gases from a copper converter difficulties have been encountered, particularly in 15 that the cost of the sulfur dioxid was too 20 high. This is due in part to the fact that in converting copper the matte ordinarily contains a relatively high percentage of iron and a small percentage of miscellaneous impurities, in addition to the copper and 25 sulfur, and therefore, in the early stages of the blowing, the air acts on the iron and other impurities as well as on the sulfur, and therefore, the gases are so low in sulfur 30 dioxid that the quantity of water required to absorb the sulfur dioxid makes the process expensive.

It has been proposed to utilize the heat of the converter gases for generating steam in 35 boilers, but here again difficulties have been encountered, because in the early stages while the iron and miscellaneous impurities are coming off, the gases carry flue dust, ejected slag and fume, which have an objectionable effect on the boiler operations.

Generally speaking, the copper matte in 40 the first stages of the converting process may contain approximately forty (40) per cent. of copper, thirty (30) per cent. of iron, twenty-five (25) per cent. of sulfur, 45 and five (5) per cent. of miscellaneous impurities. At this stage the converter gas might contain perhaps as high as fourteen (14) per cent. of sulfur dioxid, but as a practical matter, due to leakages around 50 the hood caused by frequent breaking of the hood connections, the percentage is considerably lower, not averaging over seven (7) per cent. of sulfur dioxid.

After the process has been carried on

until the matte has reached a stage where it 55 is commonly known as white metal, it may contain approximately seventy-five (75) per cent. of copper, and the balance almost all sulfur. At this stage the converter gas might run in the neighborhood of twenty- 60 one (21) per cent. of sulfur dioxid. At this stage of the operation the hood connections are not broken, but the connection cannot be made perfectly tight, and therefore there is some leakage, so that in practice this percentage might be reduced as low as fifteen 65 (15) per cent.

It will be seen, therefore, that a recovery process applied to a single converter would be acting on a gas, the composition and 70 character of which is variable, or if the process was used only when the gas was in a satisfactory condition, the process would be intermittent and the heat from the gases could not be used in boilers.

To overcome these objections I have devised a system whereby the matte is treated in one set of converters until it reaches the stage where the converter gas is of a character to permit the profitable recovery of 80 the sulfur dioxid, or in other words, until the matte has reached the stage where it is commonly known as white metal. This white metal is then removed to a separate converter, or preferably a pair of converters, 85 and the recovery process is then carried on.

In the accompanying drawing, I have shown diagrammatically a pair of converters in which the white metal is treated, and 90 the heat of the converter gases used under a pair of boilers for the purpose of reducing the cost of recovery.

The converters 1 and 11 are of the usual rotary type, and discharge their gases 95 through flues 2 and 12, provided with dampers 3 and 13, respectively. These converters are used alternately, so that while one is blowing the other is being emptied and recharged. The flues from the converters 100 join in a common passage 4, and by means of the dampers 3 and 13 a continuous flow of converter gas may be maintained through the common passage 4. From this common passage 4 lead flues 5, provided with dampers 6, to one or more boilers 7. It is desirable to use at least two boilers because if it is necessary to clean or repair a boiler it 105

can be cut out by means of its damper 8 without stopping the operation of the converters.

After the converter gas passes through 5 the boilers 7, and its heat is there utilized to the desired extent, it passes into the flue 9, where it goes on to be treated in the usual manner for the recovery of the sulfur dioxid. This process of recovery is well 10 known and need not be described.

By this means I obtain a steady flow of converter gas containing no objectionable impurities to prevent its use in boilers, and the converter gas is high enough in sulfur 15 dioxid to make the recovery process more profitable. The steam from the boilers may be used in the later stage of the recovery process.

By separating the converting process into 20 separate stages and at the same time definitely controlling one of these stages to produce a predetermined volume of gas within a practically definite time by using a fixed quantity of material of a uniform composition, I have been enabled to eliminate the 25 difficulties which have heretofore attended the recovery of sulfur dioxid from the waste gases in this class of metallurgical operations. By my improved process the losses 30 resulting from the handling of large quantities of waste gases which are low in their carbon dioxid content is avoided, and on the other hand, a constant volume of gas which has a relatively high and profitable 35 sulfur dioxogen content is obtained. Consequently the extraction of the sulfur dioxid can be carried on in subsequent operations with a uniform and constant supply of gas according to a definite plan and resulting 40 in a minimum outlay for apparatus and for operation.

Having described my invention, what I claim is:

1. The process of recovering sulfur dioxid 45 from copper matte, which consists in treating the copper matte to drive off gases having a relatively low sulfur dioxid content, then removing portions of the matte and successively blowing such portions for predetermined periods of time to maintain a 50 continuous flow of gas having a relatively high sulfur dioxid content and free from solid impurities.

2. The process of recovering sulfur dioxid 55 from copper ores, which consists in treating ores to reduce the same to matte, then treating said matte in a plurality of converters to produce white metal, removing said matte in predetermined quantities at intervals, 60 from each of said converters and subjecting such removed portions successively to an air blast for predetermined periods of time required to maintain a continuous flow of gas containing a relatively high percentage of sulfur dioxid,

3. The process of recovering sulfur dioxid from copper matte, which consists in treating the matte in a plurality of converters to obtain a supply of white metal, successively removing portions of said white metal 70 from the converters at intervals, subjecting said removed portions successively to intense heat to maintain a continuous flow of gas having a substantially uniform sulfur dioxid content and continuously collecting 75 said sulfur dioxid.

4. The process of recovering sulfur dioxid from copper matte, which consists in heating the matte to form white metal, successively removing portions of said white metal 80 at regular intervals, heating each of said portions for a predetermined time to maintain a continuous supply of gas having a relatively high percentage of sulfur dioxid and continuously collecting 85 said sulfur dioxid.

5. The process of recovering a constant supply of sulfur dioxid from converter gases, which consists in treating copper matte to produce white metal, successively 90 removing a sufficient quantity of said white metal to give off a predetermined quantity of sulfur dioxid, and successively treating said portions of white metal for predetermined periods to maintain a constant supply 95 of gas of approximately uniform composition.

6. The process of recovering a constant supply of sulfur dioxid from converter gases, which consist in treating the matte 100 to form white metal, then successively removing predetermined portions of white metal and treating the same to maintain a flow of gas of substantially constant volume containing a relatively high percentage of 105 sulfur dioxid.

7. The process of providing a constant supply of sulfur dioxid from converter gases, which consists in blowing copper matte until the gases produced therefrom have a predetermined composition, then removing portions of the matte, successively heating and blowing said portions to maintain a steady flow of gas of substantially constant volume, collecting said gases, and removing the sulfur dioxid.

8. The process of recovering sulfur dioxid from copper matte, which consists in blowing the matte until the gas produced therefrom has a predetermined composition, then 120 removing the matte to a plurality of converters, treating the matte in each converter alternately for approximately an equal period of time whereby a continuous flow of gas is obtained of substantially uniform composition.

9. The process of recovering sulfur dioxid from copper matte, which consists in collecting the gases from a plurality of converters, supplying each converter alter- 130

nately with matte adapted to produce a gas having a predetermined composition and treating the matte in each converter for approximately equal periods of time whereby 5 a continuous flow of gas may be obtained of substantially uniform composition.

10. The process of recovering sulfur dioxid from waste gases from copper matte converters which consists in treating the 10 matte in one set of converters until substantially all of the impurities except sulfur have been removed, then removing the residual matte to another set of converters, successively treating the residual matte in 15 each converter of said second set of converters for a predetermined time to maintain a constant supply of gas, passing the resultant gas through a boiler to utilize the heat, and then treating the gas to extract 20 the sulfur dioxid.

11. The process of recovering sulfur dioxid from waste gases from copper matte converters which consists in treating the

matte in one set of converters until it becomes white metal, then removing the residual matte to another set of converters and treating the same to obtain a continuous flow of gas of substantially uniform composition, passing the resultant gas through a boiler to utilize the heat, and 25 30 then treating the gas to extract sulfur dioxid.

12. The process of recovering sulfur dioxid from a pair of blocks of a sulfur containing substance such as copper matte, 35 which consists in treating the substance to drive off gases having a relatively low sulfur dioxid content, blowing first one and then the other block to maintain a continuous flow of gas having a relatively high sulfur dioxid content and collecting said high grade sulfur dioxid gas. 40

Signed at New York city, in the county of New York and State of New York, this 4th day of May, A. D. 1918.

WILLIAM H. HOWARD.